

Oct. 18, 1927.

H. F. BUSCH

1,646,187

CORK RIBBON AND METHOD OF MAKING THE SAME

Filed July 1, 1926



INVENTOR

Herman F. Busch  
by Byers, Stubbins & Hormann  
his attorney

## UNITED STATES PATENT OFFICE.

HERMAN F. BUSCH, OF MILLVALE, PENNSYLVANIA, ASSIGNOR TO ARMSTRONG CORK COMPANY, OF PITTSBURGH, PENNSYLVANIA, A CORPORATION OF PENNSYLVANIA.

## CORK RIBBON AND METHOD OF MAKING THE SAME.

Application filed July 1, 1926. Serial No. 119,927.

This invention relates to cork ribbon and method of making the same, and is particularly adapted for use in the manufacture of artificial cork ribbon in relatively long 5 lengths.

Heretofore short strips of artificial cork have been made by skiving strips from the face of a slab of artificial cork. By this method the lengths of the strips have been 10 limited to the lengths of the standard cork slabs from which they are cut, the slabs being usually about 36 inches long.

I provide a method of manufacturing artificial cork ribbon wherein substantially 15 the entire volume of a block of artificial cork may be cut into a continuous ribbon. This is accomplished by cutting the cork ribbon from the periphery of a disk or circular 20 block of artificial cork. The general type of veneer machine which is preferably employed to do this work is illustrated and described in Busch Patent No. 1,122,070 of December 22, 1914, although certain modifications of the machine may be desirable 25 to better suit this particular class of work.

My cork ribbon in its long lengths is particularly suitable for feeding to the automatic machines which cut disks therefrom and insert them as liners or washers in 30 crown bottle seals and caps for collapsible tubes. The ribbon, because of its uniform structure and thickness, is particularly adapted for making air-tight packing, such as used in player pianos. It may also be 35 used for various other purposes, such as the packing employed between the body parts of automobiles.

I preferably provide that the artificial cork ribbon has a uniform grain structure 40 throughout its length. It is desirable that the flattened granules in the artificial cork be disposed at an angle, preferably normal, to the surface of the ribbon. Ribbon having the granules disposed in this manner 45 can be cut to a more uniform thickness. Moreover, since the granules are cut transversely, there is no tendency for them to puff up or scrape off.

Referring to the accompanying drawings, 50 illustrating certain preferred embodiments of my invention,—

Figure 1 is a diagrammatic plan view

showing the method of cutting the ribbon;

Figure 2 is a side elevation of the apparatus shown in Figure 1;

Figure 3 shows a roll of the cork ribbon; and

Figure 4 is a perspective detail view of a piece of the ribbon showing the preferred grain structure.

In Figure 1, there is shown an artificial cork disk 2 secured to a mandrel 3 by suitable clamping washers 4 and nuts 5. A rotary knife 6 substantially tangentially engaging the disk 2 cuts a ribbon 7 therefrom. The circular knife 6 is carried by a shaft 8 which is suitably rotated by a source of power, not shown.

In the preferred method of making the ribbon, a standard slab of compressed artificial cork of 24 x 36 x 2 inches is first formed.

It is well known in this art that compressed artificial cork is made by compressing and setting under heat a mass consisting of granulated cork and an elastic binder. The granulated cork is screened to the desired fineness of granules, the size of the granules being dependent somewhat upon the use to which the material is to be put. Usually in making artificial cork, the granules are not more than about  $\frac{3}{2}$  inches in diameter and will pass through a screen having 11 meshes to the inch. Preferably none of the particles are fine enough to pass through a screen having 40 meshes to the inch. Usually the bulk of the material will pass through a 16 mesh and over a 28 mesh screen. The granulated cork is mixed with the binder, usually glycerine and gelatine containing a hardener such as formaldehyde.

After the materials are mixed, they are pressed in the mold to a slab, the volume being reduced to about one-eighth of the initial volume of the uncompressed mixture. During this compression the individual granules or particles of cork are flattened into small pancake shaped granules, the planes of compression of which lie, of course, normal to the direction of the compression of the cork. The slabs contained in the molds are confined under pressure and subjected to the baking operations usually employed in the manufacture of arti-

ficial cork. Artificial cork slabs and their manufacture are well known in this art and do not need to be described in greater detail.

5 The slab of compressed artificial cork is then cut lengthwise into two slabs of 12 x 36 inches. These slabs are then split to a thickness equal to the desired width of the ribbon, say  $\frac{1}{2}$  inch. The slabs  $\frac{1}{2}$  inch 10 thick are then cut into 12 inch squares, and these squares are cut into disks to be placed in the ribbon cutting machine. Other methods of forming the disks may be employed, but the procedure outlined above 15 gives good results.

I preferably provide that the standard 20 artificial cork slab be made with the planes of compression substantially parallel to the faces thereof, in order that the flattened granules comprising the slab will be disposed at a substantial angle to the edges of the slab, and hence at a substantial angle to the edges of the disks formed from the slab. Ribbon cut from the periphery of a disk 25 formed this way has a substantially uniform grain structure throughout its length, and inasmuch as the flattened granules are cut transversely, the thickness of the ribbon may be determined accurately. Furthermore, the 30 flattened granules will not subsequently tend to puff up or scale off. In some arts, for example the manufacture of pneumatic player pianos, it is highly desirable that the air packing material be of uniform 35 structure and thickness.

Figure 3 shows, to reduced scale, a roll of 40 artificial cork ribbon made according to my invention. The advantages of ribbon in this form over the strips heretofore supplied in 45 relatively short lengths are particularly pronounced when the ribbon is supplied to automatic machines. For such uses, it is of great advantage to have the cork ribbon supplied in considerable length, and it is desirable that the material be uniform.

Figure 4 shows, to enlarged scale, a small 50 portion of the ribbon 7, and clearly indicates the preferred grain structure, that is, the flattened granules are rooted in the body 55 of the ribbon, are disposed edgewise at right angles to the face of the ribbon, and are cut transversely along the face of the ribbon. The flattened granules are also disposed longitudinally of the ribbon, which arrangement, combined with their position normal 60 to the face of the ribbon, makes the ribbon structurally strong both against lengthwise 65 pull and against abrasion, as well as insur-

ing the retaining of an accurate gauge in thickness.

It will be understood, however, that the invention is not limited to cork having this 60 particular structure, since it may be desirable, in certain instances, to modify the grain structure to suit the particular use 65 to which the ribbon is to be put.

While I have illustrated and described the preferred form of my invention, it will be understood that the invention is not limited 70 to the illustrated form, but may be otherwise embodied and practiced within the scope of the following claims.

I claim:

1. An artificial cork ribbon cut from a block of compressed artificial cork, the ribbon being longer than the block from which 75 it is cut and having the flattened cork granules disposed at an angle to the face of the ribbon.

2. A ribbon of compressed artificial cork 80 having the flattened granules thereof disposed at an angle to the face of the ribbon.

3. A ribbon of compressed artificial cork 85 having the flattened granules thereof disposed substantially normal to the face of the ribbon.

4. A ribbon of compressed artificial cork having the planes of compression of the flattened granules thereof disposed longitudinally of the ribbon and substantially normal 90 to its face.

5. In the method of forming an artificial 95 cork ribbon, the steps consisting in forming a disk of compressed artificial cork wherein the flattened cork granules are disposed at a 100 substantial angle to the peripheral face of the disk, and cutting the ribbon from the peripheral face of the disk.

6. In the method of forming an artificial 105 cork ribbon, the steps consisting in forming a flat disk of compressed artificial cork wherein the planes of compression are substantially parallel to the flat face of the disk, and cutting the ribbon from the peripheral face of the disk.

7. In the method of forming an artificial 110 cork ribbon, the steps consisting in compressing the artificial cork to form a slab, cutting a disk from the slab, so that the planes of compression are substantially parallel to a flat face of the disk, and cutting a ribbon from the peripheral face of the disk.

In testimony whereof I have hereunto set my hand.

HERMAN F. BUSCH.